

## UNITED STATES PATENT OFFICE

2,515,743

ACID AFTERTREATMENT OF METALLIZED  
RESORCINOL-AZO DYES FURTHER COU-  
PLED ON THE FIBERClemens Streck, Loudonville, N. Y., assignor to  
General Aniline & Film Corporation, New York,  
N. Y., a corporation of DelawareNo Drawing. Application December 7, 1948,  
Serial No. 64,045

3 Claims. (Cl. 8—42)

**1** This invention relates to an improved process of dyeing and printing, adapted for continuous operation, yielding brown azo colorations on cellulosic materials, said colorations being developed on the fiber.

It has been suggested, as a convenient method of continuous dyeing and printing with azo dye-stuffs on cellulosic materials, to pass the material through a bath containing an azo coupling component so as to impregnate the material therewith, followed by application of a diazo component by printing or by impregnation in a second bath, and causing the diazo component to couple with the coupling component on the fiber.

One of the chief difficulties attendant upon such a process is the fact that many coupling components are substantive to the cellulosic fiber and hence, the concentration of the coupling component bath is progressively reduced as the coloring operation proceeds, resulting in a progressive decrease in the depth of the coloration. To maintain the coupling component concentration constant by progressive addition of supplemental coupling component to the bath is practically impossible, so that the aforesaid procedure is unsuitable in practice when the coupling component is substantive to the material to be dyed.

Substantivity toward cellulosic fiber (i. e. cotton and regenerated cellulose fiber or fabrics containing the same) is especially characteristic of coupling components suitable for the production of brown shades. However, the metallized o-carboxy- and o-hydroxyaryl azo resorcinols disclosed as coupling components in U. S. P. 2,135,433, which yield brown shades on cellulosic textile materials when coupled thereon with diazotized aromatic amines, constitute an exception to this general rule. These coupling components have low substantivity toward cellulosic materials, and when used in a bath for impregnating material, preparatory to development with a diazo compound thereon, the concentration of the coupling component bath remains substantially unchanged. This class of coupling components is therefore adapted in this respect for the production of uniform brown colors on cellulosic materials in continuous dyeing and printing processes of the type described above.

Nevertheless, it was found, in attempting to carry out continuous dyeing of cellulosic textile material by progressive application of the aforesaid coupling component from a bath, and subsequent development of a brown azo dyestuff on

**2** fiber by treatment with a diazonium salt, that the coloration produced varied in different parts of the material from a reddish to a yellowish shade of brown rendering the dyeing unacceptable.

A similar variation in shade resulted in printing cellulosic material grounded with the aforesaid coupling component, with a diazonium compound made up in the form of a printing paste.

**10** I have discovered that the aforesaid variation in shade can be avoided in continuous dyeing or printing processes employing said metallized o-carboxy- and o-hydroxyaryl azo resorcinols for impregnating the material, by bathing the material, after coupling is completed, with an acid solution of sufficiently strong acidity to remove alkali metal bound by the dyestuff on the fiber. After removing the acid from the material, e. g. by rinsing with water, the goods **15** can be soaped, rinsed and dried, or otherwise finished in the usual manner. The colorations thus produced are brown shades of outstanding brilliance, having excellent fastness to light, washing and similar deteriorating agencies, said colorations being uniform throughout the material.

**20** The metallized coupling components employed in accordance with my invention are metal complex compounds of o-carboxy- and o-hydroxyaryl azo resorcinols, containing in complex combination, a metal having an atomic weight between 58 and 64 (i. e. copper, nickel or cobalt) and preferably copper, said coupling components containing no other acidic salt-forming substituent (e. g. COOH or SO<sub>3</sub>H groups) in the aryl residue. The compounds have the general formula



**35** whereon Ar is an aryl radical (of which the nuclei are preferably of the benzene, naphthalene or azo-benzene series), X is a radical in o-position to the azo linkage of the class consisting of —O— and —COO—, R is a nuclear substituent of the class consisting of hydrogen and a lower alkyl group such as a methyl or ethyl group, the radical Ar containing no additional acid salt-forming substituents such as carboxyl groups or sulfonic acid groups. Substituents which may be present in the Ar radical are, for example, halogen (chlorine or bromine), nitro groups, lower alkyl groups (methyl or ethyl groups) and

sulfonamide groups ( $\text{SO}_2\text{NH}_2$ ). The metallized aryl azo resorcinols of this invention are obtained by known methods, involving coupling a diazotized o-hydroxy, o-alkoxy or o-carboxy aromatic amine of the formula  $\text{ArNH}_2$  (Ar having the same significance as in the formula given above) with resorcinol or a lower nuclear alkyl resorcinol, and subjecting the resulting azo compound in metallizing treatment, for example, by heating in an aqueous solution or suspension of a complex-forming salt, oxide, hydroxide, or carbonate of a metal having an atomic weight of 58 to 64, preferably copper.

Diazonium compounds which are suitable for production of brown shades on cellulosic materials in accordance with my invention, when combined with the aforesaid coupling components, are diazotized aromatic amines containing no acid salt-forming substituents in the aromatic radical, in the form of diazonium salts such as the chloride, acid sulfate, aryl sulfonates, and double salts of the chloride with zinc chloride, cobalt chloride, magnesium chloride or boron trifluoride. In the case of diazonium compounds of which the mineral acid salts are relatively unstable, the aforesaid double salts or aryl sulfonates are preferably used. The diazonium compounds obtained from primary aromatic amines of the benzene and biphenyl series are particularly suitable.

For impregnation of cellulosic textile materials, the coupling components of the class above described are dissolved in an aqueous alkaline solution (e. g. dilute caustic alkali solution such as aqueous sodium hydroxide). The textile material is impregnated with the coupling component solution by passing it through the bath and removing excess liquid, e. g. by passing it between squeeze-rolls. In order to dye the material, it is then passed through an aqueous solution of a diazonium salt having sufficient acidity to neutralize free alkali from the initial impregnating bath, thereby promoting coupling of the diazonium compound with the coupling component. Coupling occurs in neutral to weakly acid medium. In printing processes, the diazonium salt is made up in the form of a thickened aqueous printing paste which is printed on the material impregnated with the coupling component solution, the paste likewise having sufficient acidity to neutralize free alkali on the material and thereby effecting coupling in the printed areas.

In accordance with my invention, when coupling of the azo dye components on the material is complete, the dyed or printed goods is passed through an aqueous acid bath of sufficiently strong acidity to neutralize or remove all of the alkali metal bound by the azo dyestuff on the fiber. For this purpose, a strong acid bath is employed, preferably having a pH not greater than 2 and is preferably a dilute aqueous solution of a strong mineral acid, e. g.  $\text{HCl}$ ,  $\text{H}_2\text{SO}_4$ ,  $\text{H}_3\text{PO}_4$  or an acid salt of strong mineral acid such as sodium bisulfate. Duration of the treatment is adjusted with regard to the particular conditions of agitation and concentration so as to insure thorough penetration of the material by the acid solution. In general, a period of less than 10 minutes is sufficient. The acid solution is then removed, for example, by rinsing with water or dilute alkali, and the goods are soaped, rinsed, and dried or otherwise finished in the usual manner.

The process of my invention is illustrated by the following examples wherein parts are by weight unless otherwise indicated.

#### Example 1

7 grams of a coupling component having the following formula



10 obtained by coppering a reaction product produced by coupling diazotized 2-amino-4-chlorophenol with resorcinol, are pasted with 14 cc. of alcohol, diluted with 15 cc. of cold water and mixed with 3.5 cc. of 34° Be. sodium hydroxide solution. The resulting mixture is stirred into 1,000 cc. of water to which are added 10 cc. of 34° Be. sodium hydroxide solution and 10 cc. of Monopol oil (a soap of a highly sulfonated unsaturated fatty acid of a natural fat or oil).

15 Cotton textile material is passed progressively through the resulting bath so as to impregnate it with the solution in a continuous manner. Excess impregnating solution is squeezed off, and the material is thereupon passed through an aqueous solution containing zinc chloride double salts of 5-chloro-2-methoxy benzene diazonium chloride in a concentration of 1.075%. Coupling occurs spontaneously, the acid of the diazonium solution being sufficient to neutralize the free alkali of the coupling component solution carried by the fiber. In accordance with my invention, after the development of coloration is complete, the material is passed through an aqueous 10° Be. hydrochloric acid solution, duration of the treatment therewith being 3-5 minutes. After rinsing with water to remove the acid, the goods is soaped, rinsed and dried in the usual manner. The coloration thus produced is a uniform, rich yellow-brown shade having excellent fastness to light and washing.

#### Example 2

20 Cotton material impregnated with the coupling component solution as described in Example 1 is printed with an aqueous paste of the diazonium salt employed in the preceding example, made by replacing part of the water of the solution of Example 1 with a thickening agent such as British gum, dextrin, gum tragacanth or starch thickening to yield a printing paste of desired consistency. After development of the dyestuff on the fiber, the goods is passed through a hydrochloric acid bath and rinsed in the same manner described in the first example. Thereafter the goods can be soaped, rinsed and dried as indicated above. Brown prints are obtained of uniform shade having the outstanding fastness properties noted in the preceding example.

25 Instead of the coupling component employed in the foregoing examples, there can be substituted corresponding nickel or cobalt complex compounds of 5-chloro-2-hydroxyphenylazo resorcinol. Similarly, there can be used copper, nickel or cobalt complex compounds, but preferably the copper complex compounds, obtained by metallizing treatment of the following azo resorcinols:

- 30 5-nitro-2-hydroxyphenyl azo resorcinol
- 35 5-methyl-2-hydroxyphenyl azo resorcinol
- 40 5-chloro-2-hydroxyphenyl azo-2'-methyl resorcinol
- 45 3,3'-dimethoxy biphenyl-4,4'-bis(azo resorcinol)
- 50 4-(3'-sulfonamido-phenyl azo)-5-methyl-2-hydroxyphenyl azo resorcinol
- 55 2-hydroxynaphthyl-1-azo resorcinol
- 60 2-carboxyphenyl azo resorcinol

The resulting coppered complex compounds of the above listed materials have the following formulae



Instead of the diazonium salts disclosed in the example, other diazonium salts can be substituted, as for example, the chlorides, acid sulfates, aryl sulfonates, and zinc chloride, cobalt chloride, magnesium chloride, or boron trifluoride-diazonium chloride double salts derived from the following aromatic amines by diazotization and conversion to the aforesaid salts:

p,p'-diamino diphenylamine  
4-benzoylamino-2,5-diethoxyaniline  
dianisidine  
4-cyano-2,5-dimethoxyaniline  
p-amino-o,o'-azotoluene  
o-chloroaniline  
m-chloroaniline  
o-nitroaniline  
p-nitroaniline  
2-(4'-chlorophenoxy)-5-chloroaniline  
2,5-dichloroaniline  
4-nitro-o-toluidine

In carrying out the acid treatment of my invention, aqueous solutions of strong mineral acids such as sulfuric acid, hydrochloric acid, o-phosphoric acid, are preferably employed, for example, in concentrations up to about 20%, the amount of acid being preferably sufficient to yield a pH of not more than 2; while excessive concentrations likely to injure the fiber or decompose the dyestuffs during acid treatment are avoided. After the treatment, the acid is removed as by rinsing, and the material is finished

in the usual manner as by soaping, rinsing and drying.

Instead of the cotton goods of the example, regenerated cellulose textiles can also be dyed and printed in the same manner.

Variations and modifications which will be obvious to those skilled in the art can be made in the foregoing procedures without departing from the scope of the invention.

10 I claim:

1. In the process of coloring cellulosic material involving progressively impregnating the material by passage of the material through an aqueous alkaline solution of a coupling component of the class consisting of metal complex compounds of o-carboxy and o-hydroxy aryl-azo-resorcinols containing, in complex combination, a metal having an atomic weight between 58 and 64, said coupling component containing no other acidic salt-forming substituents, and developing an azo dye coloration for the impregnated material by applying thereto an aromatic diazonium salt containing no acidic salt-forming substituents, the improvement which comprises treating the material, after development of the azo dye coloration, with an acid solution having a pH not greater than 2, in order to convert all of the alkali bound by the dyestuff to salts of said acid; and removing the acid from the material.
2. In the process of coloring cellulosic material involving progressively impregnating the material by passage of the material through an aqueous alkaline solution of a coupling component of the class consisting of a copper complex compound of o-carboxy and o-hydroxy aryl-azo-resorcinols, said coupling component containing no other acidic salt-forming substituents, and developing an azo dye coloration on the impregnated material by applying thereto an aromatic diazonium salt containing no acidic salt-forming substituents, the improvement which comprises bathing the material, after development of the azo dye coloration, with an aqueous solution of a strong mineral acid having a pH not greater than 2, in order to convert all of the alkali bound by the dyestuff to salts of said acid; and removing the acid from the material.
3. In a process of coloring a cellulosic material involving progressively impregnating the material by passage of the material through an aqueous alkaline solution of a complex copper compound of 5-chloro-2-hydroxyphenyl azo resorcinol, and developing an azo dye on the impregnated material by applying thereto an aromatic diazonium salt containing no acidic salt-forming substituents, the improvement which comprises bathing the material, after development of the azo dye colorations thereon, with an aqueous hydrochloric acid solution having a pH not greater than 2 in order to convert all of the alkali bound by the dyestuff to a salt of said acid, and rinsing the material to remove the acid.

CLEMENS STRECK.

#### REFERENCES CITED

65 The following references are of record in the file of this patent:

#### UNITED STATES PATENTS

70 Number Name Date  
2,135,433 Delfs Nov. 1, 1938